

1

2,711,375

**PRESSURE SENSITIVE MANIFOLD SHEET**

Robert W. Sandberg, Dayton, Ohio, assignor to The National Cash Register Company, Dayton, Ohio, a corporation of Maryland

No Drawing. Application February 19, 1954,  
Serial No. 411,580

2 Claims. (Cl. 117—36)

This invention relates to a record material transfer sheet, useful in duplicating and manifolding operations, and more particularly relates to such a sheet in which the transfer coating has, therein, material which prevents smudging during ordinary handling of the paper but which in no way interferes with the transfer characteristics of the sheet.

This is a continuation in part of my application for United States Letters Patent Serial No. 243,583, filed August 24, 1951, now abandoned. In the mentioned application, of which this is a continuation in part, the invention was described with reference to a transfer coating which consisted of a hydrophilic colloid film having dispersed therethrough a profuse number of microscopic droplets of an oily marking fluid. This transfer film was derived from an oil-in-water emulsion. The outer phase of the emulsion was the film-forming colloid material, dispersed in water. The invention described in that application provided for the inclusion in the emulsion of a certain amount of microscopic cellulose fibers. Because of the nature of the emulsion, the amount of cellulose fibers which could be used was limited due to the fact that any increase of over 70% of fiber, as compared to the weight of the dried colloid material, would be deleterious to the emulsion, so that proper coating could not be made therewith. Since the filing of said application, there has been developed a coating composition which may be coated on paper to produce a manifold sheet, the coating being of hydrophilic colloid material containing oily droplets of marking fluid, but each droplet is encased in its own capsule of the colloid material, and it is derived, not from an emulsion, but from a process of coacervation, as will be explained. Because of this capsule formation on a microscopic scale, as little or as much cellulose fiber may be used to make the coating to be applied with the paper as is desired, and, hence, the limits of added fiber material set out in the application to which reference has been made are no longer important.

The invention will be described with reference both to the embodiment found in said earlier-filed application and to the embodiment in which encapsulated droplets of printing fluid from the major portion of the coating composition.

In both instances, the transfer film is rupturable by marking pressures, so as to release the oily marking fluid from the hydrophilic colloid, whether in a continuous film form or in the microscopic capsule form. In a transfer sheet having a film of the novel coating, as pressure is applied by a writing or printing instrument, the hydrophilic material is ruptured at the points of pressure, allowing the fluid to be transferred to the undersheet.

In collated forms consisting of an oversheet, the under side of which has thereon the novel transfer film in one or the other of the forms which will be described, and an undersheet to receive the transfer of material, the contact of the transfer film with the undersheet, if long continued under pressure, will result in smudging, as would be the

2

case with ordinary carbon paper. The transfer sheet provided by this invention has the cellulose fiber ingredients in the film to prevent such smudging.

The continuous-film type of transfer record material, which is the embodiment disclosed in the previous application for United States Letters Patent, to which reference has been made and of which this is a continuation in part, is disclosed in United States Letters Patent No. 2,374,862, which issued on the application of Barrett K. Green, and in United States Letters Patent No. 2,548,366, which issued on the application of Barrett K. Green and Robert W. Sandberg. In the first mentioned patent, the front surface of the record material sheet is left uncoated, and the oily material in the transfer film on the rear surface contains either coloring matter in the colored state, or colorless color-reactant material, for use on sensitized record material, which causes the appearance of color in the oil transferred thereto by reason of a color reaction. In the last mentioned patent, the front surface of the sheet of record material is coated with a sensitizing material, which causes color in a colorless color reactant applied thereto, and the rear surface has a coating containing the oil droplets of the colorless color reactant, said record sheet being useful as one of the middle sheets of a stack and acting in the capacity of both a transfer sheet and a receiving sheet.

In the second, and preferred, embodiment of the invention, as has been said, the transfer coating consists of a number of individual capsules of hydrophilic colloid material, of microscopic size, each capsule containing one or more oil droplets containing the marking ingredient. This type of manifold sheet is described in an application for United States Letters Patent, Serial No. 365,198, filed June 30, 1953, by Barrett K. Green and Lowell Schleicher.

The cellulose fibers are preferably alpha cellulose, and those used in the continuous type of film derived from an emulsion should be not more than approximately 35 microns in length, so as not to interfere with the emulsion structure. In the capsular type of coating, with which there is no danger of interfering with the emulsion, the fibers may be up to 350 microns in length or more.

Whereas in a continuous type of transfer film there may be used 7% to 70% of fibers, by weight, based on the dried colloid material without the liquid inclusions, the cellulose fibers may be used with the capsule type of transfer coating in any quantity desired, as long as the coating holds together on the paper.

Therefore, it is an object of this invention to provide a record sheet having thereon a transfer coating which includes fluid droplets of marking fluid protected from escape by film-forming hydrophilic colloid material which is rupturable by marking or printing pressures to release the oil, and which hydrophilic colloid material has incorporated therein cellulose fibers of microscopic size, which cause the transfer film to be resistant to destruction by rough handling, so as not to prematurely release the oily marking fluid.

With this and incidental objects in view, the invention includes certain novel features, the preferred and other embodiments of which are hereinafter described in this specification.

As has been said, the continuous-film type of transfer coating is an emulsion made from a sol of hydrophilic colloid material which forms the external phase, and an oily marking fluid which forms the internal phase. The cellulose fibers can be added either to the internal phase material, to the external phase material, or to both materials before they are emulsified together, or into the emulsion after the first blending of the two phases. The emulsion is more easily made by adding the cellulose fibers to the internal phase material before it is blended with the external phase material, because of the contact

3  
of said cellulose fibers with the oily internal phase material, and the method of preparing the coating will be described with that in mind.

In the continuous-film type of coating, the selected marking material is a colorless color-reactant compound, which is dissolved in a chlorinated diphenyl of approximately 48% chlorine content, and the process of making it will largely follow that disclosed in United States Letters Patent No. 2,548,366, of Barrett K. Green and Robert W. Sandberg, the novelty over such method as disclosed in said patent being the use of cellulose fibers.

The external phase material is made by incorporating one part, by weight, of animal gelatin, having an isoelectric point of pH 8 and a jelly strength of 275 grams, as measured by the Bloom gelometer, in three parts, by weight, of water, heated to 150 degrees Fahrenheit, to form a sol.

The internal phase is made by dissolving 1½ parts, by weight, of crystal violet lactone, and 1½ parts, by weight, of benzoyl leuco methylene blue in 97 parts, by weight, of chlorinated diphenyl, as specified. Alpha cellulose fiber, as specified, in an amount which will be equivalent to 4%, by weight, of the finished emulsion, is mixed into the solution which is to form the internal phase. Into four parts, by weight, of the external phase is blended three parts, by weight, of the oily internal phase material plus the added cellulose fiber. These materials are then emulsified by stirring for the required period.

The finished emulsion is applied while still hot, or reheated if it has been allowed to cool, to paper, and dried. The coating is applied in such an amount that, when dried, the coating will be of the order of .001 of an inch in thickness. As has been said, the preferred average drop size is of the order of 2½ to 3½ microns, the presence of the cellulose fiber making the drop size more uniform than would be the case if the cellulose fibers were not used. In emulsions where the cellulose fiber is not used, such might end with the spread of the internal drop size between 1 and 5 microns. As mentioned, the alpha cellulose is preferred, and the fiber length should be of the order of five to ten times the diameter of the average drop size of the internal phase, although that ratio is not critical. This emulsification takes about thirty minutes, by stirring in an open receptacle.

The specified crystal violet lactone is a colorless, or white, crystalline compound, which assumes a dark blue color on contact with acid-like clay, such as attapulgite, with which paper may be sensitized, such sensitized paper also being disclosed in the United States Patent No. 2,548,366, just mentioned. The molecular formula of crystal violet lactone is 3,3 bis (p-dimethylaminophenyl)-6 dimethylamino phthalide, and the crystal violet lactone may be made by the process disclosed in United States Letters Patent Re. 23,024, which issued on the application of Clyde S. Adams.

The benzoyl leuco methylene blue has the following structure:



and may be purchased commercially.

The emulsion coating may be air-dried at normal temperature or by a hot-air blast.

In this embodiment of the invention, the fibers of cellulose first come into contact with the oil internal phase and then become incorporated in the external phase. If desired, all or part of the cellulose fibers are put into what

is to become the external phase before the intended external phase and the intended internal phase are blended together. This results in the very satisfactory smudge-proof record material, and the required time of emulsification is reduced. If it is so desired, the cellulose fibers 5 may be beaten into the emulsion ingredients while in the emulsification stage, and they may be incorporated therein at any time up to and including the final stirring. Of course, in the latter event, the fibers play no part in 10 reducing the required emulsification time, and the finished record material made therefrom is not quite as good as that made from the emulsion of the first-described process.

Among the very many useful color-reactant compounds 15 which may be used in place of the crystal violet lactone and the benzoyl leuco methylene blue are the following:

3,3 bis (p-dimethylaminophenyl) phthalide  
3,3 bis (p-dimethylaminophenyl)-4,5,6,7 tetrachloro 20 phthalide  
3,3 bis (p-diethylaminophenyl) - 6 dimethylamino phthalide  
2,4 bis [p-(p-dimethylaminophenylazo) anilino]-6 hydroxy sym. triazine

25 Already colored compounds which may be used instead of a color-reactant compound are Sudan III; carbon black, which may be mixed with oil; Sudan IV; and oil-soluble nigrosine.

The gelatin of the external phase may be replaced by 30 polyvinyl alcohol, if desired.

Other oils that may be used in place of the chlorinated diphenyl are paraffin oil, naphthenic oil, castor oil, neat's foot oil, lard oil, olive oil, tributyl phosphate, and ethyl-phthalyl-ethyl-glycolate.

35 *The preferred embodiment, in which the transfer coating consists of microscopic capsules containing the marking oil mixed with the cellulose fiber*

40 In the preferred embodiment of the invention, the capsules containing the printing fluid are made first, and then the cellulose fibers are added with a binder, so that they are not within the colloid itself but are interlaced in and around the colloid capsules.

45 First will be described the method of making the capsules, in accordance with the application for United States Letters Patent Serial No. 365,198, of Barrett K. Green and Lowell Schleicher, filed June 30, 1953, before mentioned.

50 The encapsulating material, which encloses the oil droplets, is a complex of gelled hydrophilic colloid materials. The printing fluid of the preferred type is the crystal violet lactone mentioned in connection with the first embodiment specified above, dissolved in oil, which produces dark blue marks when coming into contact 55 with record material sensitized with clay-like material such as attapulgite, or zeolite material such as sodium aluminum silicate material.

55 In forming the capsules from a complex of gelatin and gum arabic, 20 grams of gum arabic is dissolved in 60 160 grams of water, and into that is emulsified 80 grams of trichlordiphenyl containing 3% to 6%, by weight, of the color-reactant material crystal violet lactone, and the additive material benzoyl leuco methylene blue, before mentioned, in equal amounts. The emulsification is 65 carried on until the drop size of the oil is from 2 to 5 microns. Next, 20 grams of gelatin is dissolved in 160 grams of water and mixed with the emulsion. This emulsion is then diluted by adding water uniformly and slowly, with agitation, until coacervation occurs, the complex gum arabic-gelatin colloid material forming around the droplets of the oil. These colloid-surrounded droplets make aggregates of from several microns in diameter up to 70 microns in diameter, depending upon the rate and extent of dilution. The added water should 70 amount to about 500 to 550 grams. Up to this time, all 75

the ingredients are kept at approximately 50 degrees centigrade, which is above the gel point of the ingredients. Now that the colloid material has deposited around the oil droplets, forming particles, the colloid material is caused to gel by pouring in a quantity of cold water; for instance, water at zero degrees centigrade. The mass is agitated and then let stand for one hour at not over 25 degrees centigrade. At this point, the total weight of all the ingredients should be about 3960 grams. At this point, the pH is adjusted to between 9 and 7, 10 such adjustment being made with sodium hydroxide, and the material is left for thirty minutes or more in this state. The capsules are then hardened by pouring in about 20 grams of a solution of formaldehyde in water, of about 37% formaldehyde content, and the materials are agitated for ten minutes or more at three degrees centigrade or lower. This material is adjusted to the desired water content to form a coating composition; that is to say, water may be added or taken away by filtering or centrifuging until the desired coating viscosity is obtained.

15 Into this may be added the cellulose fibers in the desired amount. Paper-coating starch may be added to act as a binder to help the cellulose fibers stick to the paper.

20 In a typical example of paper-coating composition, the solids in the paper-coating composition would consist of 100 grams of the capsules, with the included oil, taken on a dry basis—that is to say, without the water—40 grams of cellulose fiber, and 10 grams of paper-coating 30 starch. The amount of fiber is not critical, and as little or as much as desired may be used.

5 The coating composition containing the cellulose fibers is coated on paper by any of the well-known paper-coating means, as by brushing or roller-coating, and dried. As before said, the fibers may be of any size desired, fiber lengths as long as 350 microns not being appreciably noticeable in the coating.

10 While the form of the invention shown and described herein is admirably adapted to fulfill the objects primarily stated, it is to be understood that it is not intended to confine the invention to the one form or embodiment disclosed herein, for it is susceptible of embodiment in various other forms.

What is claimed is:

15 1. A manifold sheet having a coating thereon of pressure-rupturable hydrophilic colloid material enclosing microscopic discrete liquid inclusions of an oily marking substance and the coating containing microscopic fibers of cellulose isolated from the liquid inclusions, and said fibers being present in an amount not to exceed 70% by weight based on the dried colloid material without the liquid inclusions and not exceeding 35 microns in length.

20 2. A manifold sheet having thereon a coating of pressure-rupturable microscopic capsules of hydrophilic colloid material, each capsule containing an oily marking fluid and the coating containing interlaced around the capsules microscopic fibers of cellulose.

References Cited in the file of this patent

UNITED STATES PATENTS

2,655,453 Sandberg ----- Oct. 13, 1953